

## UNITED STATES PATENT OFFICE

2,297,932

## PRINTING PLATE PREPARATION

William H. Wood, Bedford, Ohio, assignor to  
 Harris-Seybold-Potter Company, Cleveland,  
 Ohio, a corporation of Ohio

No Drawing. Application August 31, 1940,  
 Serial No. 355,024

8 Claims. (Cl. 95—7)

In the manufacture of ordinary lithographic printing plates the usual practice is to coat the plate, generally of zinc or aluminum, with an aqueous solution of albumen sensitized by the addition of ammonium bichromate. The coating is allowed to dry, is exposed to light to form the desired image, then coated with developing ink and the unhardened albumen is removed with water, leaving hardened albumen in those areas which correspond to the image to be printed. In the manufacture of so-called "deep-etch" lithographic plates, a light-sensitized "resist" is employed which usually consists of an aqueous solution of gum arabic or gum arabic and dextrose to which ammonium bichromate has been added. The plate is coated with this solution, is allowed to dry, and is exposed to light forming the desired image, and the unhardened areas are removed by development with water, leaving hardened coating as a protective resist over the non-image areas of the plate. An etching solution, as for instance iron chloride is then employed to eat away the unprotected image parts of the plate to a desired depth. The etched parts are then filled with an ink receptive lacquer, ink is applied, and the hardened protective resist is removed by dilute citric acid solution leaving the plate clean in the unetched non-image areas. In the manufacture of half-tone relief plates and some forms of intaglio plates, while in many instances a shellac resist or "cold top enamel" is applied and the plate is etched by nitric acid, it is also common to make such plates by means of materials similar to those just mentioned for deep etch lithographic plates, viz. gum arabic and dextrose resist and iron chloride etching solution. In relief plates the resist protects the image areas from the action of the etching fluid and in intaglio plates the resist protects the non-image areas. In both cases the resist is removed after etching by suitable means to prepare the plate for printing. Some other practices are occasionally employed, varying in details and in materials. All, however, are characterized in that a colloidal material sensitized to light is carried by the plate, and is exposed to light corresponding to the image or non-image areas, as the case may be, in accordance with the subject matter to be reproduced, and the unhardened areas or coating are removed and the plate is used for printing, either directly with the hardened areas of coating remaining thereon, or by etching the plate and thereafter removing the hardened areas. In accordance with the present invention, it now becomes possible to produce

plates such as afore-mentioned, with surfacing which presents advantages over such substances as albumen, gum arabic, dextrose, etc. previously involved.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

In accordance with the invention, a solution for plate coating is prepared, of arabogalactan. A convenient and desirable solvent is water, arabogalactan being a known polysaccharide, and usually assigned the formula



derived in one mode of manufacture from wood, and being in its commercial state a dry, white, light-weight powder, and its molecular weight being around 2500, dissolving in water much more readily than albumen or gum arabic, and going into solution almost immediately whereas albumen or gum arabic usually requires soaking in water for several hours. It forms clear colorless solutions which may be of very high concentration or as desired. Such solutions have a notably lower viscosity than albumen or gum arabic solutions of the same concentration, and this is of particular advantage in permitting attainment of uniform relatively thick coatings of the dried material on the plates. As a basis for coatings, the arabogalactan being produced as a chemical product is further advantageous in affording controllable uniformity in grade, unlike the variations in such natural products as albumen and gum arabic.

The aqueous solution of arabogalactan of desired concentration for coating the plates is applied in suitable manner, and a light sensitizing agent is provided, such as a chromate or bichromate, and most conveniently this may be included in the solution before coating the plates. Where desired, the plates may however be coated with the arabogalactan solution and dried, and the sensitizing agent may be applied subsequently, as for instance in alcoholic solution. The proportions of the ingredients are not critical and in general may be similar to those employed in albumen and gum arabic solutions. However, and particularly where a thicker coating is desired, the proportion of arabogalactan

may be increased to any degree consistent with the results desired. The plates or place to which the coating is applied, may be of the customary character and metals, zinc, aluminum, etc.

As an example of the manufacture of ordinary lithographic plates, a solution comprising about 10 per cent of arabogalactan and about 3 per cent of ammonium bichromate in water, is applied to the plates, and the sensitized coating is allowed to dry. The plates are exposed to a light image in the usual way, and developing ink is then applied and the unexposed portions are removed with water, leaving the hardened exposed portions of the arabogalactan coating on the plate in ink-receptive condition. The developed plate is then treated with a de-sensitizing solution of usual or preferred composition for rendering the non-printing areas ink-repellent and water-receptive. The plate may then be put on the press for printing. Such a plate comprises printing areas formed of arabogalactan hardened by light action.

As an example of the preparation of deep etched lithographic plates, a water solution comprising about 20 per cent of arabogalactan and about 6 per cent of ammonium bichromate is coated onto the plates, and after drying, the plates are exposed to light corresponding to the non-image areas of the subject. The unexposed coating is removed by dissolving with water, and the plate is etched with the usual iron chloride and lactic acid solution or other preferred solution, and lacquer and ink are applied as usual. The hardened resist is then removed with dilute citric acid solution, and the non-image areas are de-sensitized to ink, and the plate may then be used for printing.

As an example of the manufacture of copper half-tone relief or intaglio plates, a solution comprising about 10 per cent arabogalactan and about 3 per cent ammonium bichromate is coated onto the plates and treated similarly as in the example preceding. The etching action however, is carried further to provide pronounced elevations or depressions and make up the printing surface.

Other modes of applying the principle of the

invention may be employed, change being made as regards the details described, provided the features stated in any of the following claims, or the equivalent of such, be employed.

5. I therefore particularly point out and distinctly claim as my invention:

1. As a light-sensitized material for photographic and printing purposes an aqueous solution of arabogalactan and a light-sensitizing agent capable of acting thereon.

2. As a new article of manufacture, a plate for printing usage, comprising a metal supporting base portion and a surface thereon embodying arabogalactan and a light-sensitizing agent.

15 3. As a new article of manufacture, a plate for printing usage, comprising a metal supporting base portion and a surface thereon embodying arabogalactan and a light-sensitizing chromic acid compound.

20 4. As a new article of manufacture, a plate for printing usage, comprising a surface of arabogalactan and a light-sensitizing chromic acid compound.

5. As a new article of manufacture, a plate for 25 printing usage, comprising a base and a surface coating thereon of arabogalactan and a light-sensitizing agent capable of acting on the arabogalactan.

6. As a light-sensitized material for photographic and printing purposes, an aqueous solution of arabogalactan and a light-sensitizing chromic acid compound.

30 7. As a new article of manufacture, a plate for printing usage, comprising a base and a surface coating on said base having areas for reproduction and embodying hardened arabogalactan resulting from the action of a light-sensitizing agent capable of acting thereon and exposure to actinic rays.

40 8. As a new article of manufacture, a plate for printing usage, comprising a base and a surface coating on said base having areas for reproduction and embodying hardened arabogalactan resulting from the action of a light-sensitizing 45 chromic acid compound and exposure to actinic rays.

WILLIAM H. WOOD.